

# UNITED STATES PATENT OFFICE.

CLARENCE ROSCOE KING, OF WORCESTER, MASSACHUSETTS, ASSIGNOR TO NORTON COMPANY, A CORPORATION OF MASSACHUSETTS.

## PROCESS OF MAKING FILLED ABRASIVE WHEELS.

1,187,431.

Specification of Letters Patent. Patented June 13, 1916.

No Drawing.

Application filed May 28, 1914. Serial No. 841,679.

To all whom it may concern:

Be it known that I, CLARENCE ROSCOE KING, a citizen of the United States, residing at Worcester, in the county of Worcester and State of Massachusetts, have invented a new and useful Process of Making Filled Abrasive Wheels, of which the following is a specification.

This invention relates to a process of making filled abrasive wheels and particularly to the process of making a filled wheel having certain distinguishing characteristics.

The details of my improved process are fully described in the following specification and the novel features thereof will be specifically defined in the appended claims.

I have discovered that when certain types of abrasive wheels are filled with a material having certain definite characteristics, the efficiency of the wheels as grinding tools is thereby greatly increased. The increase in efficiency is most marked when this treatment is applied to abrasive wheels having a porous unitary structure, such wheels being ordinarily formed by uniting loose grains of abrasive material by some form of silicate binder.

The most common types of these wheels are commercially known as vitrified wheels and silicate wheels. In the first class, the silicate binder is composed largely of clay mixed with other mineral silicates, this mixture being partially fused when burned in a kiln and thus forming a porous mass in which the abrasive particles are securely held, the bond partaking largely of the nature of porcelain or glass. In the silicate wheels, the principal binding material is silicate of soda commonly known as "water glass." This silicate, when mixed with certain mineral powders and heated to a sufficient temperature, reacts with the other materials and forms a hard porous mass similar in many respects to the vitrified wheels.

In the use of these wheels in grinding the efficiency of the abrasive is reduced by glazing and also by the filling or loading of the wheel. The term "glazing" is used to indicate the action of the work upon the abrasive particles by which they lose their sharp edges and become smooth and ineffective, while the term "loading" relates to the filling up of the voids in the face of the wheel by particles of the material being

ground, this loading of the face causing the cutting edges of the abrasive to be covered. I have discovered that the efficiency of such a wheel may be greatly increased by filling the voids of the porous structure with some material which is normally solid but which becomes fluid and sticky at the temperatures ordinarily attained in the grinding operation. While there are a considerable number of materials possessing these characteristics, I have found that ordinary rosin is particularly well adapted for the purpose stated.

In the carrying out of my improved process, I form an abrasive wheel, preferably with a silicate binder, and having a porous unitary structure. In order that the voids of the wheels may be thoroughly filled I heat the wheel to a temperature substantially the same as that of the melted rosin and then dip the wheel in the rosin. I have found it advantageous to allow the wheel to remain in the rosin bath for a considerable period of time, usually about one hour, so that all of the voids in the structure may be thoroughly filled with the liquid rosin. I then remove the wheel from the rosin bath and allow it to cool until the rosin is solidified within the voids.

In order that the filling material may be evenly distributed throughout the structure I find it advisable to frequently turn the wheels during the cooling process. This result may be attained by mounting the wheel upon an arbor and slowly revolving it thereon or by laying the wheel upon its flat side and frequently reversing its position. I have proved by actual tests that the efficiency of an abrasive wheel is increased in a most remarkable degree by this treatment. As the rosin is solid at ordinary temperatures and is very sticky at grinding temperatures the wheels thus treated will not get out of balance by the flowing of the rosin from one portion to another.

The action of the filling material upon the cutting operation has not been determined with absolute certainty but it apparently forms a sticky film upon the grinding surface which takes up the stock as it is removed from the work and thus prevents its becoming embedded in the voids of the wheel. This thin film quickly cools as it leaves the working point and when cooled

it is so brittle that it may be dislodged and thrown off during the revolution of the wheel.

While I have described the use of rosin for carrying out my invention I do not wish to be limited thereto as I have previously pointed out that any ingredient having the characteristics of being normally solid at ordinary temperatures and of becoming fluid and sticky under the heat attained in the grinding operation is adapted for use in my improved process. It will be evident also that the filling material may be applied to the wheel by other means than dipping the wheel in the material and I do not wish to be limited to any particular procedure in carrying out the process except as pointed out in the following claims.

Having thus described my invention what I claim and desire to secure by Letters Patent is:—

1. The process of making a filled abrasive wheel which consists in forming an abrasive wheel with a silicate binder and having a porous unitary structure, heating said wheel to a moderate temperature, dipping said

wheel into a hot melted material which is solid at ordinary temperatures and becomes fluid and sticky at grinding temperatures and thereafter cooling said wheel.

2. The process of making a filled abrasive wheel which consists in forming an abrasive wheel with a porous unitary structure, heating said wheel to a moderate temperature, filling the voids in said wheel with a hot melted material which is solid at ordinary temperatures but becomes fluid and sticky at the temperatures attained in grinding, removing and cooling said wheel to solidify said material, and slowly turning said wheel during the cooling operation so that the absorbed filling material may be retained within the wheel and may be distributed with substantial uniformity throughout the porous structure.

In testimony whereof I have hereunto set my hand, in the presence of two subscribing witnesses.

CLARENCE ROSCOE KING.

Witnesses:

CHAS. T. HAWLEY,  
C. FORREST WESSON.